

## 1

3,427,153

**METHOD OF PREPARING ALLOY BLACKS**  
Peruvamba Swaminatha Venkatesan, Bronx, and Melvin  
Yarish, Brooklyn, N.Y., assignors to Leesona Corpora-  
tion, Warwick, R.I., a corporation of Massachusetts  
No Drawing. Filed June 11, 1964, Ser. No. 374,274  
U.S. Cl. 75—108 2 Claims  
Int. Cl. C22c 1/06, 5/00

## ABSTRACT OF THE DISCLOSURE 10

An improved method of preparing alloy blacks is de-  
scribed. The method comprises admixing salts of the  
desired metals of the alloy in the proper ratios, forming  
a co-precipitate of the metals by addition of ammonium  
hydroxide to the salt solutions, and reducing the co-pre-  
cipitated hydroxide.

This invention relates to the preparation of alloy blacks  
in finely divided form. More particularly, the invention  
relates to a simplified method for the preparation of im-  
proved alloy blacks. Basically, the improved method com-  
prises admixing salts of the desired metals of the alloy  
in the proper ratios, forming a precipitate of the metal  
alloy by addition of ammonium hydroxide and reducing  
the co-precipitated hydroxide.

It is recognized in the art that many metals, particularly  
the transition metals of the fifth and sixth series of  
Group VIII of the Mendelejeff's Periodic Table and the  
noble metals of Sub-Group I have excellent properties as  
catalysts particularly in gas-solid reactions. Quite sur-  
prisingly, when certain alloys of two or more metals are  
prepared, the alloys have enhanced catalytic properties in  
comparison with any of the metals of the alloy taken  
singly. Therefore, the use of alloys as catalysts has be-  
come more prevalent in recent years, particularly as acti-  
vators in fuel cell electrodes, i.e., cells wherein the energy  
of reaction between a fuel and an oxidant is converted  
directly into electrical energy.

Further, it is known that the value of a catalyst, apart  
from the intrinsic activity of the material, is directly re-  
lated to the surface area of the catalyst exposed to re-  
actants. For this reason, metals and alloys are used as  
catalysts in finely divided or spongy form having a high  
surface area. Although there are several methods of pre-  
paring finely divided metals such as electrolytic precipita-  
tion of the metal from a suitable salt solution, the prepa-  
ration of alloy blacks presents more of a problem. Thus,  
one method of preparing blacks of an alloy is first to  
form an alloy by known metallurgical means such as melting  
powders of the different metals together in the proper  
proportions, preferably above the melting point of the  
metals and thereafter cooling. The alloy is formed into  
wires or narrow strips by usual methods known in the art  
such as drawing, etc. The alloy wires or strips are mounted  
in ice water as electrodes, i.e., as an anode and cath-  
ode. A direct current potential of between 150 and 200  
volts is applied to the system and the wires brought into  
close proximity to establish an arc. The arcing disrupts  
the metals and forms a fine suspension of alloy particles  
in the water. The metal particles are filtered out, dried,  
and employed in known procedures. As apparent, the  
above-described process is complex and time consuming.

It has now been found that alloy blacks can be pre-  
pared by forming admixtures of the desired metal salts  
in their proper ratio, adding ammonium hydroxide to the  
admixture to form the co-precipitated metal hydroxides  
and thereafter reducing the metal hydroxide with a reduc-  
ing agent, such as hydrazine or bubbling hydrogen, to  
form the alloy blacks. In addition to the aforesaid process

## 2

being extremely simple, the blacks formed have enhanced  
activity particularly when used on fuel cell electrodes,  
possibly due to an increase in the surface area.

Accordingly, it is an object of the present invention  
to provide an improved method of preparing metal alloy  
blacks.

It is still a further object of the present invention to  
provide metal alloy blacks having a large surface area by  
forming admixtures of the metal salts in the desired ratio,  
co-precipitating the metal hydroxides by adding ammonium  
hydroxide and reducing the co-precipitate.

It is a still further object of the present invention to  
provide gold-palladium alloy blacks by adding a solution  
of ammonium hydroxide to an aqueous solution of pal-  
ladium and gold salts to form the co-precipitated hydro-  
xides and thereafter reducing with an aqueous hydrazine  
solution to form the finely divided metal alloy black.

These and other objects of the invention will become  
more fully apparent from the following detailed descrip-  
tion and illustrative examples.

The alloy blacks of any of the noble metals such as  
the so-called platinum and palladium metals and gold  
and silver can be prepared according to the method of the  
present invention. Thus, it is merely necessary to admix  
salts of the desired metals in the proper ratio and there-  
after form the hydroxides and reduce. However, although  
metal alloy blacks of ruthenium, rhodium, palladium,  
osmium, iridium, platinum, gold, and silver can be pre-  
pared, gold-palladium alloy blacks are preferred in view  
of their exceptional activity and stability, particularly  
when employed as a catalyst on a fuel cell electrode.

The admixtures of metal hydroxides can be prepared  
from aqueous salt solutions of the metals, such as solu-  
tions of the chlorides, nitrates, and sulfates. However,  
it is necessary that the precipitate be prepared from a  
solution of the two or more metals of the alloy. Thus,  
quite surprisingly, it was found that when gold and  
palladium were precipitated separately, and thereafter  
the precipitates admixed and reduced, an alloy was not  
obtained but merely an admixture of the two metals. The  
temperatures at which the precipitated hydroxides are  
formed or reduced are not critical and can be varied  
over a substantially wide range.

The alloy blacks can be used in any of the areas where  
conventional blacks have been employed.

Having described the invention in general terms, the  
following example is set forth to illustrate a preferred  
embodiment of the invention.

## EXAMPLE

An alloy black was prepared by dissolving gold chlo-  
ride salt in a concentrated aqueous palladium chloride  
solution, the concentration in terms of metal being 100  
mg./ml., to obtain a gold to palladium ratio of 75:25  
on an atomic percent basis. The mixture was introduced  
slowly into a 3% ammonical solution at room tempera-  
ture with constant stirring. Upon contact of the two solu-  
tions, a finely divided yellow precipitate was formed im-  
mediately. Thereafter, an excess of dilute hydrazine was  
added to reduce the precipitated material to the finely  
divided metallic state. After washing in distilled water  
and drying, tests showed the finely divided metallic par-  
ticles to be the gold-palladium alloy.

To demonstrate the utility of the novel alloy black,  
a reducing electrode was prepared by coating a nickel  
scale with a paste prepared from the above-described al-  
loy black and Teflon suspended in water. The Teflon,  
having an average particle size of 0.3 micron in diameter,  
and the alloy black were present in a ratio of 3:10. After  
coating the screen with the paste, the system was stabil-  
ized by heating at 300° C. for 30 minutes. After cooling,

the Teflon gold-palladium alloy coating adhered very well to the support screen.

The structure described as above was employed as the cathode in a fuel cell in conjunction with a similarly constructed anode employing platinum black as the activator. The electrolyte of the cell is a 5 normal aqueous potassium hydroxide solution. The operating temperature is 75° C. The anode is fed with hydrogen at a pressure of 0.15 p.s.i.g. Oxygen is fed to the cathode at a pressure of 0.25 p.s.i.g. Current density versus cell potential data are as follows:

| Current density (ma./cm. <sup>2</sup> ): | Cell potential<br>(volts) |
|------------------------------------------|---------------------------|
| 0                                        | 1.092                     |
| 40                                       | .965                      |
| 80                                       | .945                      |
| 120                                      | .931                      |
| 180                                      | .913                      |
| 240                                      | .894                      |
| 300                                      | .882                      |
| 400                                      | .859                      |

In the aforesaid examples, the palladium and gold can be replaced by combinations of other metals such as platinum, ruthenium, osmium, iridium, silver, and rhodium. Such combinations must be capable of forming mixed oxide and/or hydroxide phases and solid metal solutions or an intermetallic phase. Moreover, the percentages of the different metals in the alloy can be varied to obtain substantially different compositions. Other metal salts can be employed in the preparation of the metal hydroxides. It should be appreciated that the invention is not to be limited by the example as it is possible to pro-

duce still other embodiments without departing from the inventive concept herein disclosed and covered by the appended claims.

What is claimed is:

5. The method of preparing a palladium-gold alloy black comprising the steps of (1) adding gold chloride to an aqueous solution of palladium chloride to obtain the desired gold to palladium ratio, (2) forming a precipitate by adding ammonium hydroxide to the solution of (1), and (3) reducing said gold and palladium hydroxide precipitate with hydrazine to form a metal alloy black.

10. The method of preparing a metal alloy black comprising the steps of (1) forming a solution of at least two metal salts; (2) forming a co-precipitate of the metals by adding ammonium hydroxide to the salt solution; and (3) reducing said co-precipitated metal hydroxide with a member of the group consisting of hydrazine and bubbling hydrogen to form a metal alloy black.

#### References Cited

#### UNITED STATES PATENTS

|              |         |               |       |        |
|--------------|---------|---------------|-------|--------|
| 2,254,976    | 9/1941  | Powell        | ----- | 75—108 |
| 2,375,506    | 5/1945  | Turck         | ----- | 75—108 |
| 25 2,726,151 | 12/1955 | Kern          | ----- | 75—108 |
| 2,787,540    | 4/1957  | Appell        | ----- | 75—108 |
| 2,863,762    | 12/1958 | Pullen        | ----- | 75—108 |
| 2,970,051    | 1/1961  | Mackiw et al. | ----- | 75—108 |

30 RICHARD O. DEAN, *Primary Examiner.*

U.S. Cl. X.R.

75—118, 121